

Jan. 8, 1929.

1,698,669

C. F. BRUSH, JR

PIEZO ELECTRIC CRYSTALS

Original Filed May 6, 1927

FIG. 1.



FIG. 2.



FIG. 3.



FIG. 4.



FIG. 5.



FIG. 6.



FIG. 8.



FIG. 9.



Inventor.

Charles F. Brush, Jr.

By Evans & McCoy

Attorneys

## UNITED STATES PATENT OFFICE.

CHARLES F. BRUSH, JR., OF CLEVELAND HEIGHTS, OHIO; THE CLEVELAND TRUST COMPANY, EXECUTOR OF SAID BRUSH, JR., DECEASED, ASSIGNOR, BY MESNE ASSIGNMENTS, TO THE CLEVELAND TRUST COMPANY, OF CLEVELAND, OHIO, A CORPORATION OF OHIO.

## PIEZO-ELECTRIC CRYSTALS.

Application filed May 8, 1927, Serial No. 189,440. Renewed June 15, 1928.

This invention relates to piezo-electric crystals and more particularly to a method of improving the characteristics of piezo-electric crystals, such as Rochelle salt crystals of the 5 composite type.

The term "composite crystal" as applied to piezo-electric crystals, particularly Rochelle salt crystals, relates to the type of crystal having opaque or porous end regions. The term 10 "hour-glass" is also frequently applied to this structure due to the shape of the opaque regions. These regions are, in fact, of irregular crystalline structure containing occluded mother liquor and are the result of rapid 15 growth of the crystal and may be produced, for example, by allowing the temperature of a saturated aqueous solution of Rochelle salt to fall comparatively rapidly. If the solution from which such crystals are 20 deposited be allowed to cool more slowly, this hour-glass structure is less marked and may be eliminated entirely by extremely slow cooling. These hour-glass regions contain mother liquor even after extensive desiccation 25 of the crystal. Thus, after soaking the crystal in absolute alcohol for several days and then baking for a week at 40 degrees C. these hour-glass regions are still moist as may be demonstrated by cutting open the 30 crystal. More violent desiccation, such as heating in vacuo, will dry up these regions to some extent. It has long been observed, however, that these hour-glass regions were necessary for the successful operation of this type 35 of crystal.

In electrical work, as in sound reproducing mechanism, a pair of terminals is usually secured to each such crystal. One such terminal usually or frequently comprises a pair 40 of connected electrodes pressed against the porous or hour-glass ends of the crystal, the other terminal being formed by a metal foil band substantially encircling the body of the crystal, as is well known in the art. The 45 crystal is then frequently coated with an insulating material, such as a varnish. The crystal is then frequently mounted in a cradle, one end of the crystal being pressed against or otherwise fixedly attached to the 50 cradle, the other end of the crystal being attached to a lever arm pivoted with respect to the cradle. With such mounting, as is well

known, a potential applied to the electrodes will produce a torsional stress in the crystal and consequent movement of the lever arm, 55 and vice versa. With respect to such devices, the moist hour-glass regions of the crystal are electrically conductive and thus form inner electrodes which have been found necessary for the successful operation of devices 60 of this type.

Certain serious disadvantages accompany the use of such crystals. Thus, for example, the relatively highly electrically conductive porous or hour-glass regions tend to dry up 65 by spontaneous evaporation, with accompanying decrease in electrical conductivity and consequent decrease in piezo-electrical activity. A further difficulty has been caused by leakage of the liquid from the hour-glass 70 region, particularly after the crystal has been subjected to violent electrical or mechanical stresses for relatively long periods. Such leakage liquid has frequently crept around the outside of the crystal beneath an 75 insulating coating, such as varnish, whereby to short-circuit the apparatus. Moreover, the porous or hour-glass regions are at best somewhat irregular and non-uniform in extent and character. Such irregularities 80 result in non-uniform electrical performance and sometimes result in electrical puncture due to the breaking down of the crystalline structure intermediate an hour glass portion and an electrode, by the difference of electric 85 potential between said electrode and the porous or hour-glass region.

An object of my invention is to provide a method of treating piezo-electric crystals to provide a crystal structure of a high degree of 90 uniformity and efficiency.

Another object of this invention is to provide a method of treating piezo-electric crystals to form crystal structures of uniform and permanent character.

A further object of my invention is to provide a method whereby the porous or hour-glass regions of a composite Rochelle salt crystal may be permanently rendered highly 95 electrically conductive.

Another object of the invention is to provide a piezo-electric crystal having conductive portions of permanent and uniform character.

A further object of my invention is to provide a composite Rochelle salt piezo crystal having improved electrical characteristics.

Another object of this invention is to provide a piezo-electric crystal of increased efficiency.

Other objects of the invention will be apparent from the description of it hereinafter given, and the accompanying drawings, 10 wherein

Figure 1 is a top plan view, and Fig. 2 is a perspective view, of a composite Rochelle salt crystal before being treated according to my invention;

15 Fig. 3 is a bottom plan view of a composite Rochelle salt crystal, showing apertures through the base thereof;

Fig. 4 is a sectional view illustrating one 20 form of apparatus in which my invention may be carried out;

Fig. 5 is a bottom plan view of a composite Rochelle salt crystal after being treated according to my invention; metal foil being shown associated with the crystal;

25 Fig. 6 is a horizontal sectional view on line 6-6 of Fig. 7, showing a crystal from which material has been removed, one of the cavities being filled with conductive material, the other cavity being lined with conductive material;

Fig. 7 is a vertical section on line 7-7 of Fig. 6;

Fig. 8 is a plan view of an acoustic device 30 embodying a crystal treated according to my invention; and

Fig. 9 is a front elevation of the structure shown in Fig. 8.

My invention may be said to comprise generally the increase of permanency and efficiency of crystals of the type described by 40 rendering the hour-glass regions of such crystals permanently and uniformly electrically conductive. It will be understood, of course, that the beneficial results of my invention 45 may be obtained in various ways.

One manner in which my invention may be carried out contemplates removing the liquid material from the hour-glass regions 1 of a crystal 2 and substituting therefor 50 conducting material which can neither dry up nor leak out. Thus, for example, referring particularly to Figs. 3 and 4, there is shown a Rochelle salt crystal 2 of the composite type in which apertures 3 have been drilled in the base of the crystal so as to communicate with the hour-glass regions 1. In Fig. 4 the crystal 2 is shown as disposed on a suitable gasket 4 disposed within an air-tight chamber 5 provided with a compressed 55 air inlet 6 and an outlet 7. The crystal 2 is preferably so disposed that the apertures 3 are in substantial register with the outlet aperture 7, which outlet communicates with the atmosphere. By introducing compressed air through the inlet pipe 6 into the cham-

ber 5, the liquid in the hour-glass regions 1 is forced out of the crystal 2 through the apertures 3. The removal of the liquid from the regions 1 may frequently be facilitated by heating the crystal to a suitable temperature, such as, for example, about 40 degrees C. 70

It may be noted that the removal of the liquid from the hour-glass regions 1 renders such portions substantially electrically non-conductive, and accordingly a crystal which 75 has been so treated is relatively inactive piezo-electrically.

The hour-glass portions 1 may be rendered permanently and uniformly electrically conductive by disposing therein suitable conductive material. Such material may be introduced into the portions 1 by removing the crystal 2 from the chamber 5, disposing the material to be introduced adjacent the outer ends of the portions 1, and applying vacuum 80 to the apertures 3. The material to be introduced is accordingly sucked into the portions 1 and will fill substantially all the space previously occupied by the liquid, such as mother liquor, previously removed. 85

A suitable material for the above-described purpose is an aqueous solution of silver nitrate, which solution, if desired, may contain ammonia. After the introduction of such silver nitrate solution into the portions 1 the crystal may be exposed to light whereby metallic silver will be precipitated within the portions 1. Any remaining solution may then be removed in the manner described for the removal of the original liquid contained 100 in the portions 1, or such solution may be removed by applying vacuum to the apertures 3, and subsequently drying the portions 1 by forcing air therethrough. 105

It will be understood, of course, that any 110 suitable liquid may be introduced into the portions 1 from which liquid a conductive precipitate may be deposited.

It will be further understood that there 115 may be introduced into the portions 1 a liquid which is in itself conductive but which has the property of drying and becoming non-conductive electrically when exposed to the air. Thus, for example, certain varnishes may be introduced into the portions 1 with 120 very satisfactory results. Thus, if material such as a varnish should leak out from the portions 1, such material would dry and become a non-conductor electrically, at the same time sealing the portions 1 and preventing evaporation and solidification of the material contained therein. 125

If an electrode, such as the tin foil electrode 9, is disposed about a crystal treated as hereinbefore mentioned, it will be understood that such electrode should be cut away as indicated at 10 in Fig. 5 to avoid contact with the conductive interior of the crystal 2. The slight reduction in electrode area caused by the apertures 10, however, has no 130

noticeable effect on the piezo-electric performance of the crystal.

My invention may be carried out by mechanically removing all or a portion of the hour-glass portions 1 and mechanically introducing therein conducting material to form inner electrodes. Thus, in Figs. 6 and 7, the hour-glass portions are shown as mechanically removed to form the cavities 11 and 12. 10 The cavity 11 is shown as substantially entirely filled with suitable conducting material 13 such as tin foil, amalgam, powdered graphite, or the like. The cavity 12 is shown as lined with a suitable material such as tin foil 14 to form a conductive inner electrode. In any given crystal any or all of the cavities may be provided with electrodes of the type shown at 13 or at 14.

This method of carrying out my invention 20 is advantageous in that the extent of the original hour-glass portions 1 is of no great importance, since the cavities formed by mechanical removal need not coincide with the original hour-glass portions, but may be of 25 greater or lesser extent. If of lesser extent, the hour-glass material remaining may be rendered non-conductive by heating the crystal 2 in vacuo, thereby eliminating any danger of electrical puncture as indicated above. If 30 the cavity formed by removing the portions 1 is greater in extent than the original portions 1, the piezo-electric activity of the crystal is increased due to the greater extent of the conductive material. By carrying out the 35 invention in this manner, therefore, it is possible to make the electrodes 13 or 14 of the size, shape and character most suitable for the purpose for which the crystal is to be used, regardless of the original extent of the hour-glass regions 1.

In Figs. 8 and 9 I have shown an acoustic device embodying a crystal treated according to my invention. Thus, the crystal 2 is shown as disposed in cooperative relation with the cradle 15. At each end of the crystal are shown plastic electrically conductive portions 16 and 17 disposed adjacent the electrically conductive end regions 18 and 19 of the crystal 2. The portion 17 is disposed in closely engaging position with the arm 20 of the cradle 15 whereas the portion 16 is secured to the lever arm 21 which is pivoted with respect to the cradle 15 by means of the pivot arm 22. The terminal 23 is shown secured to the foil band 9, the terminal 24 being connected to the conductive portions 16 and 17. With this construction a potential applied to the terminals 23 and 24 will produce a torsional stress in the crystal 2 and consequent movement of 55 the lever arm 21 and vice versa.

It will thus be seen that by my invention I have provided a method of treating composite crystals of the type described whereby to produce piezo-electric crystals of the desired

electrical characteristics, and of permanent 65 character and greatly increased efficiency.

It will moreover be noted that I have provided a method of producing composite crystals of the type described having predetermined electrical characteristics. 70

It will also be seen that by my invention composite piezo-electric crystals of the type described may be formed of uniform and permanent character.

It will also be noted that by my invention 75 the electrical conductivity of the hour-glass portions of piezo-electric crystals of the type described may be greatly increased and rendered permanent in character.

To those skilled in the art many modifications of and widely differing embodiments and applications of my invention will suggest themselves without departing from the spirit and scope thereof. My disclosures and the descriptions herein are purely illustrative 85 and are not intended to be in any sense limiting.

What I claim is:

1. The method of providing a piezo-electric crystal of improved characteristics which 90 comprises removing material from the ends of said crystal and associating with said ends electrically conductive material of substantially permanent character.

2. The method of improving the characteristics of a composite crystal of the type described having a region containing occluded liquid, which comprises removing material from said region, and substituting therefor other electrically conductive material. 95

3. The method of improving the characteristics of a composite crystal of the type described having a region containing liquid, which comprises removing material from said region, and substituting therefor solid 100 electrically conductive material.

4. The method of improving the characteristics of a composite crystal of the type described having a region containing liquid, which comprises removing said liquid from 110 said region and substituting therefor electrically conductive material.

5. The method of improving the characteristics of a composite crystal of the type described having a region containing liquid, 115 which comprises removing the liquid substantially completely from said region, removing a portion of said region, and substituting for said removed portion material of substantially constant electrical conductivity. 120

6. The method of improving the characteristics of a composite crystal of the type described having a region containing liquid, which comprises removing liquid from said region, introducing into said region a solution capable of yielding an electrically conductive precipitate, precipitating an electrically conductive material from said solu- 125

tion, and removing the excess solution whereby the precipitated conductive material will remain in said region.

7. The method of improving the characteristics of a composite crystal of the type described having a region containing liquid, which comprises removing said liquid sub-

ducing into said region a silver nitrate solution, precipitating an electrically conductive material from said solution, and removing the excess solution whereby the precipitated conductive material will remain in said region.

In testimony whereof I affix my signature.

CHARLES F. BRUSH, JR.